

## UNITED STATES PATENT OFFICE

2,459,116

## MINERAL OIL COMPOSITION

Edward A. Oberright, Woodbury, N. J., assignor  
to Socony-Vacuum Oil Company, Incorporated,  
a corporation of New York

No Drawing. Application July 6, 1945,  
Serial No. 603,594

8 Claims. (Cl. 252—42.7)

1

This invention has to do in a general way with mineral oil compositions and is more particularly related to compositions comprised of mineral oil and a minor proportion of an added ingredient which will improve the oil in one or more important respects.

It is well known to those familiar with the art that mineral oil fractions refined for their various uses are in and of themselves usually deficient in one or more respects so that their practical utility is limited even in the particular field for which they have been refined. For example, mineral oil fractions refined for use as lubricants have a tendency to oxidize under conditions of use, with the formation of sludge or acidic oxidation products; also, the lighter fractions such as gasoline and kerosene tend to oxidize with the formation of color bodies, gum, etc. In order to prevent the formation of these products and thereby extend the useful life of the oil fraction, it is common practice to blend with such oil fraction an additive ingredient which will inhibit oxidation, such ingredients being known to the trade as oxidation inhibitors, antioxidants, sludge inhibitors, gum inhibitors, etc.

It is also the practice to add other ingredients to mineral oil fractions for the purpose of improving "oiliness" characteristics and the wear-reducing action of such mineral oils when they are used as lubricants, particularly when the oils are used for the purpose of lubricating metal surfaces which are engaged under extremely high pressures and at high rubbing speeds.

Various other ingredients have been developed for the purpose of depressing the pour point of mineral oil fractions which have been refined for use as lubricants. Most refining treatments provide oils containing a small amount of wax which, without the added ingredient, would tend to crystallize at temperatures which render the oil impracticable for use under low temperature conditions. Additive agents have also been developed for improving the viscosity index of lubricating oil fractions. In the case of internal combustion engines, particularly those operating with high cylinder pressures, there is a decided tendency for the ordinary lubricating oil fractions to form carbonaceous deposits which cause the piston rings to become stuck in their slots and which fill the slots in the oil ring or rings, thus materially reducing the efficiency of the engine. Ingredients have been developed which, when added to the oil, will reduce this natural tendency of the oil to form deposits which interfere with the function of the piston rings.

2

It has also been discovered that certain types of recently-developed hard metal alloys, such as cadmium-silver alloy bearings, are attacked by ingredients in certain types of oils, particularly oils of high viscosity index obtained by various methods of solvent refining. This corrosive action on such alloys has led to the development of corrosion inhibitors which may be used in solvent-refined oils to protect such bearing metals against this corrosive action.

In the lighter mineral oil fractions, such as those used for fuel purposes, particularly in internal combustion engines, it has been found that the combustion characteristics of the fuel may be controlled and improved by adding minor proportions of various improving agents thereto.

The various ingredients which have been developed for use in mineral oil fractions to improve such fractions in the several characteristics enumerated above are largely specific to their particular applications. Therefore, it has been the practice to add a separate ingredient for each of the improvements which is to be effected.

The present invention is predicated upon the discovery of a group or class of oil-soluble reaction products or compounds which, when added to mineral oil fractions in minor proportions, will improve the oil fractions in several respects.

The novel addition agents contemplated by this invention as multi-functional improvers for mineral oils are oil-soluble, sulfur-containing reaction products obtained by reacting elementary sulfur or a sulfur halide, or a mixture thereof, with a condensation product of an aldehyde, a heterocyclic amine and a hydroxyaromatic compound (and metal salts thereof), the condensation products and their corresponding metal salts being represented by the general formula:



45 wherein A is an aromatic nucleus, either mono- or poly-cyclic; R' is either hydrogen or an alkyl, aralkyl, alkaryl, aryl, cycloalkyl, alkoxy or aroxy group; a represents the number of R' groups attached to an aromatic nucleus A and is an integer from 0 to 4; X is a substituent such as an amino, nitro, hydroxyl, carboxyl, or halogen group or the like; b represents the number of X groups attached to an aromatic nucleus A and is either 0 or 1; M is either hydrogen or metal; Y

50

55 is a secondary heterocyclic amine group, attached

at a secondary (heterocyclic) nitrogen atom to the carbon atom of a



group; and  $c$  represents the number of



groups attached to an aromatic nucleus  $A$  and is an integer from 1 to 3. It will be clear that when  $A$  is a phenyl nucleus, the sum of  $a$ ,  $b$  and  $c$  will not exceed 5; and when  $A$  is a naphthalene nucleus or other poly-cyclic nucleus, the sum may exceed 5.

Aldehydes contemplated by the present invention are the aliphatic aldehydes, typified by formaldehyde (such as trioxymethylene), acet-aldehyde, and aldon (B-hydroxy butyraldehyde); aromatic aldehydes, representative of which is benzaldehyde; heterocyclic aldehydes, such as furfural; etc. The aldehyde may contain a substituent group such as hydroxyl, halogen, nitro and the like; in short, any substituent which does not take a major part in the reaction. Preference, however, is given to the aliphatic aldehydes, formaldehyde being particularly preferred.

The secondary heterocyclic amines are those characterized by attachment of a hydrogen atom to a nitrogen atom in the heterocyclic group. Representative of the amines contemplated herein are morpholine, thiomorpholine, pyrrole, pyrrolidine, indole, pyrazole, pyrazoline, pyrazolidine, piperidine, phenoxyazine, phenothiazine and their C-substituted analogs. Substituent groups, attached to the carbon atoms of these amines are typified by alky, aryl, alkaryl, aralkyl, cycloalkyl, etc. Preferred of these amines is morpholine.

Representative hydroxyaromatic compounds contemplated by the present invention are phenol, resorcinol, hydroquinone, catechol, cresol, xylenol, hydroxydiphenyl, benzylphenol, phenylethylphenol, phenol resins, methylhydroxydiphenyl, guiacol, alpha and beta naphthol, alpha and beta methylnaphthol, tolylnaphthol, xylylnaphthol, benzylnaphthol, anthranol, phenylmethylnaphthol, phenanthrol, monomethyl ether of catechol, methoxyphenol, phenoxyphenol, chlorphenol, and the like. Preference in general is to the monohydroxy phenols otherwise unsubstituted, particular preference being given to phenol and alpha and beta naphthol.

The hydroxyaromatic compounds may also contain one or more substituent groups such as carboxyl, metal carboxylate, halogen, nitro, amino and the like; here again, any substituent which does not take a predominant part in the condensation with the aldehyde and the heterocyclic amine. Preferred of such substituents are carboxyl and metal carboxylate groups.

As indicated hereinabove, the hydroxyaromatic compound may contain one or more alkyl substituents, such as short-chain groups typified by methyl, ethyl, amyl, etc.; or long-chain, relatively high molecular weight hydrocarbon groups having at least twenty carbon atoms, typified by alkyl groups derived from petroleum wax, which is a predominantly straight-chain aliphatic hydrocarbon of at least twenty carbon atoms. It will be obvious to those skilled in the art that the maximum number of alkyl groups is limited by

the number of valences on the aromatic nucleus available for substitution. Naturally, the maximum number of such groups which can be attached to a single aromatic nucleus will vary as

5 the nucleus is mono- or poly-cyclic and as the nucleus is otherwise substituted, with such groups as carboxy, nitro, amino, halogen and the like.

6 A typical, and also preferred, alkyl-substituted hydroxyaromatic compound which may be used is a wax-substituted phenol, "wax-phenol." The term "wax" as used herein designates petroleum wax or aliphatic hydrocarbons or hydrocarbon groups of the type which characterize petroleum wax. These so-called "wax" substituents may be obtained by alkylation of the phenol or hydroxyaromatic hydrocarbon with a relatively high molecular weight aliphatic hydrocarbon or mixture of such hydrocarbons (such as petroleum wax) by any suitable alkylation procedure such, for example, as by a Friedel-Crafts condensation of chlorinated petroleum wax with phenol.

7 The condensation products are believed to be formed in the manner indicated in the following equation, wherein formaldehyde, phenol and morpholine are used as illustrations:



8 In preparing the condensation products, the reactants may be added to each other in any order. A typical procedure involves adding the aldehyde to an alcohol solution of the hydroxyaromatic compound and the heterocyclic amine. 9 The reaction may also be carried out in the presence of other diluents or solvents such, for example, as benzol, chlorbenzene, tetrachlorethane, mineral oil, etc. In the event that mineral oil is used as a diluent, the mineral oil may be retained, rather than separated from the condensation product, thereby providing a mineral oil concentrate which may be reacted with a sulfurizing agent. Oil concentrates of the sulfur-containing reaction products, and metal salts thereof, are similarly obtained.

10 The reaction temperature may be varied considerably, depending upon the time of reaction, the specific reactants used, etc. For example, the reaction can be carried out at 20-25° C. for a relatively long period of time or at the reflux temperature of the reaction mixture over a comparatively short period. By way of illustration, the reactants in quantities such as shown in the following example, may be thoroughly mixed at 20-25° C. for several hours and the reaction completed at the reflux temperature of the reaction mixture for an additional period of several hours.

11 The condensation product may be water washed to assure complete removal of any unreacted amine and this is recommended when the amine is high boiling. In general, however, the procedure involves distilling off the solvent which also removes any unreacted amine; water of reaction and water added with the reactants

(formaldehyde, for example, is generally used in a 37% aqueous solution).

The ratio of the reactants used may be varied to provide one or more methylene heterocyclic-amine groups,



in the condensation product. When equimolecular quantities of reactants are used, it is believed that one such group is introduced. With one mol of a hydroxyaromatic compound and two mols of amine and two mols of aldehyde, two such groups are generally introduced providing two positions, such as two positions ortho to the hydroxyl group of the hydroxyaromatic compound, or one ortho and one para thereto, are not substituted with groups other than hydrogen.

Metal salts of the condensation products may be prepared by any of the well-known procedures for replacing a hydroxyl or carboxyl hydrogen or both. Typical methods include: addition of an alcohol solution of a metal oxide or hydroxide to the condensation product; addition of a metal alcoholate in alcohol solution to the condensation product; addition of an alcohol solution of a metal salt to the sodium salt of the condensation product followed by removal of the alcohol and the sodium salt formed by double decomposition; etc.

As indicated hereinabove, the reaction products contemplated herein are prepared by reacting a condensation product of the type described above with elementary sulfur, a sulfur-halide or a mixture thereof. This reaction is preferably carried out in the presence of an inert diluent such as tetrachlorethane, benzene, chlorbenzene, mineral oil, etc. These diluents—except heavy mineral oils—are removed after the reaction by distillation of the reaction mixture which contains the desired reaction product. When mineral oil is used as the diluent, however, it may be retained, thereby providing a mineral oil concentrate containing the reaction product.

The reaction temperature may be varied considerably, depending upon the reaction time and the specific sulfurizing reactant used. Generally, higher reaction temperatures and longer reaction times are required when elementary sulfur is used than when a sulfur halide is used. The preferred procedure involves adding the sulfurizing reactant to the condensation product at 20-25° C. and thereafter heating the reaction mixture so formed at the reflux temperature of the diluent for several hours. Preference is given the sulfur halides and, of these, sulfur monochloride is particularly preferred.

Metal salts of the aforesaid sulfur-containing reaction products, as indicated above, also fall within the scope of the present invention. Any metal may be used the oxide or hydroxide of which (in alcohol solution, if necessary) can be reacted with the intermediate condensation product, or a salt of which can be reacted in alcohol solution with the sodium salt of the intermediate product. Among the metals contemplated for this purpose are: copper, beryllium, magnesium, calcium, strontium, barium, radium, zinc, cadmium, mercury, germanium, tin, lead, vanadium, chromium, manganese, iron, cobalt, nickel, ruthe-rium, palladium, platinum, aluminum, antimony, arsenic, bismuth, cerium, columbium, gallium, gold, indium, iridium, molybdenum, osmium, rubidium, selenium, tantalum, tellurium, thorium,

titanium, tungsten, uranium, and zirconium. Preference is given to metals of the alkaline earth group, particularly to barium. As noted above, the metal is preferably introduced by reaction of its oxide or hydroxide with the intermediate condensation product. Where necessary, an alcohol solution of the oxide or hydroxide is used. The metal salts can also be prepared by reacting the sodium salt of the intermediate product with an alcohol solution of a salt of the desired metal, such as stannous chloride, lead acetate, thorium nitrate, titanium tetrachloride, etc.

These metal salts may be prepared by any of the procedures referred to hereinabove for introducing metal into the intermediate or reaction products.

The sulfur-containing reaction products are illustrated by the following typical example.

#### EXAMPLE

20 Fifty grams of wax-phenol (2-18), prepared as described in U. S. Patent No. 2,191,499, and 7.7 grams of morpholine were dissolved in butyl alcohol, and 14.6 grams of Formalin (37%) were 25 added dropwise thereto, addition taking about 20 minutes. The reaction mixture thus obtained was stirred for 2½ hours at room temperature, 20-25° C., and thereafter heated at reflux, 110° C., for 8 hours. Benzol was added to the reaction mixture and was removed therefrom, with butyl alcohol and water of reaction and added water of the Formalin used, by distillation to a maximum temperature of 160° C. at 10 mms. pressure. The reaction product thus obtained was 35 wax hydroxy benzyl morpholine (2-18); nitrogen analysis revealed 1.7% nitrogen, compared with a theoretical nitrogen content of 2.0%.

30 Forty grams of wax hydroxy benzyl morpholine (2-18) was blended in 80 grams of mineral oil (S. U. V. of 65 seconds at 210° F.) and Stoddard Solvent. Four grams of sulfur monochloride in chlorbenzene were added slowly during a 30 minute period to the mineral oil-Stoddard Solvent blend, being introduced below the liquid surface. 40 The reaction mixture thus obtained became viscous whereupon additional chlorbenzene was added thereto. There was no evolution of HCl gas and, for this reason, the reaction mixture was washed with sodium acetate solution to remove any HCl associated with an amino group. Thereafter, the reaction mixture was filtered through Hi-Flo clay and the filtrate therefrom was distilled to a maximum temperature of 180° C. at 10 mms. pressure, thereby removing Stoddard Solvent and chlorbenzene. The reaction product—Product One—is a 1:2 mineral oil blend and contains nitrogen and sulfur.

45 As stated hereinbefore, the reaction products contemplated by this invention and illustrated by the above example, when added to lubricating oils in minor proportions, have been found to improve these oils in several important respects. This phenomenon is demonstrated by the following tables, which give the results of the various tests conducted to determine the effectiveness of these reaction products as addition agents for lubricating oils. The per cent of material added to the oil in the following tables is the per cent of concentrated material and does not include the oil in which the product was made.

#### POUR POINT DEPRESSION

50 Tests were conducted in the conventional manner to determine the A. S. T. M. pour points of 55 blends of these reaction products with a Mid-

Continent solvent-refined oil of S. U. V. of 67 seconds at 210° F. as compared with the pour point of the blank oil. The results given in Table I below demonstrate the effectiveness of the reaction products contemplated herein as pour point depressants.

Table I

| Addition Agent | Per Cent | A. S. T. M.<br>Pour Point<br>Values<br>°F. |
|----------------|----------|--------------------------------------------|
| None           |          | +25                                        |
| Product One    | 1/2      | -20                                        |
| Do             | 1/4      | -15                                        |

## SOCONY-VACUUM TURBINE TEST

Twenty-five cc. samples of a furfural-refined Rodessa crude of S. U. V. of 150 seconds at 100° F. and of a blend of this same oil and typical reaction products were subjected to the following test to determine the effectiveness of the reaction products contemplated by this invention as inhibitors for turbine oils: To each sample were added 1 gram of iron granules and 24 inches of 18 gauge copper wire. The samples were then heated to a temperature of 200° F. with 5 liters of air per hour bubbling therethrough. Two cc. of distilled water were added each day. The results of the tests which were made for color and acidity or neutralization number and amount of sludge formed after certain time intervals are set forth in Table II below.

Table II

| Addition Agent | Per Cent<br>Added | Hours      | Lovibond<br>Color | N. N.       | Sludge<br>(in mgms.) |
|----------------|-------------------|------------|-------------------|-------------|----------------------|
| None           |                   | 162        | 245               | 17.8        | 389                  |
| Product One    | 1/10              | 139<br>332 | 1.5<br>44         | nil<br>10.6 | 21<br>68             |

## OPERATION TEST

To demonstrate the effectiveness of the reaction products under actual operating conditions of an automotive engine, unblended oils and improved oils, containing the reaction products, were subjected to the Lauson engine test. The tests were carried out in a single-cylinder Lauson engine operated continuously over a time interval of 16 hours with the cooling medium held at a temperature of about 212° F., and the oil temperature held at about 280° F. The engine was operated at a speed of about 1830 R. P. M. At the end of each test the oil was tested for acidity (N. N.) and viscosity. The base oil used here is a solvent-refined oil having an S. U. V. of 44 seconds at 210° F.

Table III

| Addition Agent | Per Cent<br>Added | S. U. V. at<br>210° F. | N. N. |
|----------------|-------------------|------------------------|-------|
| None           |                   | 52.2                   | 7.2   |
| Product One    | 1/2               | 47.9                   | 2.9   |

It will be apparent from the foregoing test data that the characterizing materials of this invention are effective multifunctional oil improving agents.

The improved properties obtained and the degree of improvement effected may be varied with the aldehyde, heterocyclic amine, hydroxyaromatic compound, sulfurizing agent and metal

used in their preparation and present in the reaction product.

The amount of improving agent used varies with the mineral oil fraction with which it is blended and with the properties desired with the final oil composition. These reaction products, and the metal salts thereof, may be added to mineral oil in amounts of from about 0.01% to about 10%, but amounts of 0.1-5% generally provide satisfactory improvement.

It is to be understood that although I have described certain preferred procedures which may be followed in the preparation of the novel reaction products contemplated herein as multifunctional addition agents for mineral oils and have indicated representative reactants for use in their preparation, such procedures and reactants are merely illustrative and the invention is not to be considered as limited thereto or thereby but includes within its scope such changes and modifications as fairly come within the spirit of the appended claims.

I claim:

1. An improved mineral oil containing a small proportion, sufficient to inhibit said oil against the deleterious effects of oxidation, of an oil-soluble, sulfur-containing reaction product obtained by reacting (1) two molar equivalents of a condensation product of the general formula



in which A is an aromatic nucleus; R' is selected from the group consisting of hydrogen, alkyl, aralkyl, alkaryl, aryl, cycloalkyl, alkoxy and aroxy groups; a represents the number of R' groups attached to the aromatic nucleus A and varies from 0 to 3; M is selected from the group consisting of hydrogen and metal; R<sup>2</sup> is selected from the group consisting of hydrogen, alkyl, alkaryl, aralkyl, cycloalkyl and aryl groups; Y is a secondary heterocyclic amine group attached at the nitrogen atom thereof to the carbon atom of the



group; and c represents the number of



groups attached to the aromatic nucleus A and varies from 1 to 3; with (2) about one molar equivalent of a sulfurizing material selected from the group consisting of elementary sulfur, a sulfur halide and a mixture thereof, in the presence of an inert diluent, at a temperature falling within the range varying between about 20° C. and the reflux temperature of the diluent and for a time sufficient to effect sulfurization of said condensation product.

2. An improved mineral oil containing a small proportion, from about 0.01 per cent to about 10 per cent, of an oil-soluble, sulfur-containing reaction product obtained by reacting (1) two molar equivalents of a condensation product of the general formula



in which A is an aromatic nucleus; R' is selected

from the group consisting of hydrogen, alkyl, aralkyl, alkaryl, aryl, cycloalkyl, alkoxy and aroxy groups;  $a$  represents the number of  $R'$  groups attached to the aromatic nucleus A and varies from 0 to 3; M is selected from the group consisting of hydrogen and metal;  $R^2$  is selected from the group consisting of hydrogen, alkyl, alkaryl, aralkyl, cycloalkyl and aryl groups; Y is a secondary heterocyclic amine group attached at the nitrogen atom thereof to the carbon atom of the



groups attached to the aromatic nucleus A and varies from 1 to 3; with (2) about one molar equivalent of a sulfurizing material selected from the group consisting of elementary sulfur, a sulfur halide and a mixture thereof, in the presence of an inert diluent, at a temperature falling within the range varying between about 20° C. and the reflux temperature of the diluent and for a time sufficient to effect sulfurization of said condensation product.

13. An improved mineral oil containing a small proportion, sufficient to inhibit said oil against the deleterious effects of oxidation, of an oil-soluble, sulfur-containing reaction product obtained by reacting (1) two molar equivalents of a condensation product of the general formula



in which A is an aromatic nucleus;  $R'$  is selected from the group consisting of hydrogen, alkyl, aralkyl, alkaryl, aryl, cycloalkyl, alkoxy and aroxy groups;  $a$  represents the number of  $R'$  groups attached to the aromatic nucleus A and varies from 0 to 3; M is selected from the group consisting of hydrogen and metal;  $R^2$  is selected from the group consisting of hydrogen, alkyl, alkaryl, aralkyl, cycloalkyl and aryl groups; Y is a secondary heterocyclic amine group attached at the nitrogen atom thereof to the carbon atom of the



group; and  $c$  represents the number of



groups attached to the aromatic nucleus A and varies from 1 to 3; with (2) about one molar equivalent of a sulfur halide, in the presence of an inert diluent, at a temperature falling within the range varying between about 20° C. and the reflux temperature of the diluent and for a time sufficient to effect sulfurization of said condensation product.

4. An improved mineral oil containing a small proportion, sufficient to inhibit said oil against the deleterious effects of oxidation, of an oil-soluble, sulfur-containing reaction product ob-

tained by reacting (1) two molar equivalents of a condensation product of the general formula



in which A is an aromatic nucleus;  $R'$  is selected from the group consisting of hydrogen, alkyl, aralkyl, alkaryl, aryl, cycloalkyl, alkoxy and aroxy groups;  $a$  represents the number of  $R'$  groups attached to the aromatic nucleus A and varies from 0 to 3; M is selected from the group consisting of hydrogen and metal;  $R^2$  is selected from the group consisting of hydrogen, alkyl,

15 alkaryl, aralkyl, cycloalkyl and aryl groups; Y is a secondary heterocyclic amine group attached at the nitrogen atom thereof to the carbon atom of the



group; and  $c$  represents the number of



groups attached to the aromatic nucleus A and varies from 1 to 3; with (2) about one molar equivalent of sulfur monochloride, in the presence of an inert diluent, at a temperature falling within the range varying between about 20° C. and the reflux temperature of the diluent and for a time sufficient to effect sulfurization of said condensation product.

5. An improved mineral oil containing a small proportion, sufficient to inhibit said oil against the deleterious effects of oxidation, of an oil-soluble, sulfur-containing reaction product obtained by reacting (1) two molar equivalents of a condensation product of the general formula



in which A is an aromatic nucleus;  $R'$  is selected from the group consisting of hydrogen, alkyl, aralkyl, alkaryl, aryl, cycloalkyl, alkoxy and aroxy groups;  $a$  represents the number of  $R'$  groups attached to the aromatic nucleus A and varies from 0 to 3; M is selected from the group consisting of hydrogen and metal;  $R^2$  is selected from the group consisting of hydrogen, alkyl,

55 alkaryl, aralkyl, cycloalkyl and aryl groups; Y is a secondary heterocyclic amine group attached at the nitrogen atom thereof to the carbon atom of the



group; and  $c$  represents the number of



groups attached to the aromatic nucleus A and varies from 1 to 3; with (2) about one molar equivalent of elementary sulfur, in the presence of an inert diluent, at a temperature falling within the range varying between about 20° C. and the reflux temperature of the diluent and for a time sufficient to effect sulfurization of said condensation product.

70

6. An improved mineral oil containing a small proportion, sufficient to inhibit said oil against the deleterious effects of oxidation, of an oil-soluble, sulfur-containing reaction product obtained by reacting (1) two molar equivalents of a condensation product of the general formula



in which A is an aromatic nucleus; R' is a paraffin wax hydrocarbon group containing at least twenty carbon atoms; a represents the number of R' groups attached to the aromatic nucleus A and varies from 0 to 3; M is selected from the group consisting of hydrogen and metal; R<sup>2</sup> is selected from the group consisting of hydrogen, alkyl, alkaryl, aralkyl, cycloalkyl and aryl groups; Y is a secondary heterocyclic amine group attached at the nitrogen atom thereof to the carbon atom of the



group; and c represents the number of



groups attached to the aromatic nucleus A and varies from 1 to 3; with (2) about one molar equivalent of a sulfurizing material selected from the group consisting of elementary sulfur, a sulfur halide and a mixture thereof, in the presence of an inert diluent, at a temperature falling within the range varying between about 20° C. and the reflux temperature of the diluent and for a time sufficient to effect sulfurization of said condensation product.

7. An improved mineral oil containing a minor proportion, sufficient to inhibit said oil against the deleterious effects of oxidation, of an oil-soluble, sulfur-containing reaction product obtained by reacting about two molar equivalents of a paraffin wax-hydroxy-benzyl morpholine with about one molar equivalent of sulfur monochloride, in the presence of an inert diluent, at a temperature falling within the range varying between about 20° C. and the reflux temperature of the diluent and for a time sufficient to effect sulfurization of said paraffin-wax-benzyl morpholine.

8. An improved mineral oil containing a small proportion, sufficient to inhibit said oil against

the deleterious effects of oxidation, of an oil-soluble, sulfur-containing reaction product obtained by reacting (1) two molar equivalents of a condensation product of the general formula



in which A is an aromatic nucleus; R' is selected from the group consisting of hydrogen, alkyl, alkaryl, aryl, cycloalkyl, alkoxy and aroxy groups; a represents the number of R' groups attached to the aromatic nucleus A and varies from 0 to 3; R<sup>2</sup> is selected from the group consisting of hydrogen, alkyl, alkaryl, aralkyl, cycloalkyl and aryl groups; Y is a secondary heterocyclic amine group attached at the nitrogen atom thereof to the carbon atom of the



group; and c represents the number of



groups attached to the aromatic nucleus A and varies from 1 to 3; with (2) about one molar equivalent of a sulfurizing material selected from the group consisting of elementary sulfur, a sulfur halide and a mixture thereof, in the presence of an inert diluent, at a temperature falling within the range varying between about 20° C. and the reflux temperature of the diluent and for a time sufficient to effect sulfurization of said condensation product.

EDWARD A. OBERRIGHT.

#### REFERENCES CITED

The following references are of record in the file of this patent:

#### UNITED STATES PATENTS

| Number    | Name           | Date          |
|-----------|----------------|---------------|
| 2,263,445 | Reiff          | Nov. 18, 1941 |
| 2,282,710 | Dietrich       | May 12, 1942  |
| 2,322,379 | McCleary       | June 22, 1943 |
| 2,334,594 | Zimmer         | Nov. 16, 1943 |
| 2,336,006 | Fuller         | Dec. 7, 1943  |
| 2,340,036 | Zimmer         | Jan. 25, 1944 |
| 2,353,192 | Sargent et al. | July 11, 1944 |
| 2,363,134 | McCleary       | Nov. 21, 1944 |

**Certificate of Correction**

Patent No. 2,459,116.

January 11, 1949.

**EDWARD A. OBERRIGHT**

It is hereby certified that error appears in the printed specification of the above numbered patent requiring correction as follows:

Column 12, line 30, claim 8, after the word "from" insert *the group*;  
and that the said Letters Patent should be read with this correction therein that the same may conform to the record of the case in the Patent Office.

Signed and sealed this 14th day of June, A. D. 1949.

[~~MAIL~~]

**THOMAS F. MURPHY,**  
*Assistant Commissioner of Patents.*